

# United States Patent [19]

Kambara et al.

[11] Patent Number: 4,540,646

[45] Date of Patent: Sep. 10, 1985

[54] METHOD OF DEVELOPING AN ELECTROSTATIC LATENT IMAGE

[75] Inventors: Jun Kambara; Yuzo Ohmuro; Nin-ichi Kamogawa, all of Hachioji, Japan

[73] Assignee: Konishiroku Photo Industry Co., Ltd., Tokyo, Japan

[21] Appl. No.: 628,767

[22] Filed: Jul. 9, 1984

[56]

References Cited

U.S. PATENT DOCUMENTS

|           |         |                   |           |
|-----------|---------|-------------------|-----------|
| 3,345,294 | 10/1967 | Cooper .....      | 430/106.6 |
| 3,627,682 | 12/1971 | Hall et al. ..... | 430/106.6 |
| 3,639,245 | 2/1972  | Nelson .....      | 430/106.6 |
| 3,645,770 | 2/1972  | Flint .....       | 430/106.6 |
| 3,909,258 | 9/1975  | Kotz .....        | 430/106.6 |
| 3,947,370 | 3/1976  | Miller .....      | 430/106.6 |

Primary Examiner—Roland E. Martin

Attorney, Agent, or Firm—Jordan B. Bierman

Related U.S. Application Data

[60] Continuation of Ser. No. 326,588, Dec. 2, 1981, which is a division of Ser. No. 832,019, Sep. 9, 1977, which is a division of Ser. No. 608,274, Aug. 27, 1975, abandoned.

[30] Foreign Application Priority Data

Aug. 28, 1974 [JP] Japan .....

49-99385

[51] Int. Cl.<sup>3</sup> .....

G03G 13/09

[52] U.S. Cl. .....

430/122; 430/106.6;

430/903

[58] Field of Search .....

430/106.6, 107, 122,

430/903

[57]

ABSTRACT

Method and apparatus for developing electrostatic latent images comprising a developer which in turn is composed of a toner made up of resin and particles of magnetic materials having negative triboelectricity with respect to the resin dispersed in said resin. The developer is fed to a surface having magnets associated therewith for causing the developer to rise from the magnets in ear-like fashion to brush and deposit the developer on the latent image carrying surface.

9 Claims, 5 Drawing Figures



Fig. 1



Fig. 2



Fig. 3



Fig.4



Fig.5



**METHOD OF DEVELOPING AN  
ELECTROSTATIC LATENT IMAGE**

This application is a continuation of application Ser. No. 326,588 filed 12/2/81. Which is a division of our co-pending application Ser. No. 832,019 filed Sept. 9, 1977 which in turn was a division of abandoned application Ser. No. 608,274 filed Aug. 27, 1975, both of which claimed the priority of Japanese 99385/1974 filed Aug. 28, 1974.

This invention relates to a method and a device of developing electrostatic latent images, and especially a development method using a one-component type developer consisting of a toner alone.

Among the methods for developing electrostatic latent images which have heretofore been generally used for machines utilizing electrophotography of electrostatic recording, there are known a magnetic brush method, a cascade method, a wet development method and the like. Each of these developing methods is advantageous in that images of good quality can be obtained, but two-component type developers used in these methods, bring about such defects as fatigue of carriers and change in the toner content in the developer.

A number of developing methods using one-component type developers containing a toner alone and being free of carrier particles have been disclosed, and among such developing methods, there are known a touch-down method, an impression method, a fur brush method, a powder cloud method, an electrostatic induction method using a conductive toner, and the like. However, none of these methods has been used practically. The magnetic dry development method which is combined in some of office copying machines recently marketed by a few companies is a development method included in the above-mentioned electrostatic induction method, and in this development method, there is employed a conductive and ferromagnetic toner which is detailed in West German Laid-Open Patent Specification No. 2,313,297. This method is advantageous in that electrostatic latent images of either negative polarity or positive polarity can be developed by the same toner. However, because the toner is of conductive nature, when once developed images are transferred on, for example, white paper, the sharpness of the images is degraded and images of good quality can hardly be obtained. In order to overcome this disadvantage, the image transfer is practically conducted according to a method in which the transfer paper is contacted with a photosensitive layer by a conductive roller applied with an electric voltage, without adopting a customary corona discharge transfer method. This transfer method using a conductive roller, however, involves relatively troublesome problems, that, difficulty in changing the size (width) of transfer paper and requiring a mechanism for pressing the roller against the photosensitive layer surface and separating the roller from the photo-sensitive layer surface.

Accordingly, practical and excellent development methods using an insulating toner are now eagerly desired in the art. It is therefore an object of this invention to satisfy this desire. Namely, it is a primary object of this invention to provide a development method using a novel one-component type developer free of carrier particles, which method can provide images of high

quality. Particularly, the sharpness of the image is not degraded even by corona discharge transfer.

Briefly, the development method of this invention is characterized in that a toner prepared by incorporating a suitable amount of a ferromagnetic fine powder in toner particles so that a vast number of faces of such powder are exposed on the surfaces of these toner particles is used as the developer, and the development method can be performed conveniently by giving positive and negative charges to the toner particles by the triboelectric effect among the particles and forming ears composed of a plurality of the toner particles by a magnet. Accordingly, a simplified magnetic development apparatus can be used for practice of this invention and supply of the toner can be performed by very simple means. Moreover, the toner to be used in this invention is required to have specific peculiar properties not possessed by conventional toners. Namely, the toner should have sufficiently high triboelectric chargeability and good ear-forming property, and since no carrier particles are employed, the toner should have good flowability.

This invention is very unique and epoch-making in that the functions performed by the two components, that is a toner and a carrier, in the conventional techniques, are performed exclusively by a toner alone. Further, the effects attained by this characteristic feature are superior to those attained in any of conventional development methods and the method of this invention is advantageous over any of the conventional methods especially as regards simplification of the apparatus and easy maintenance thereof.

One function of a carrier, for example, iron powder used in the conventional magnetic brush development method, namely the function of imparting charges to toner particles and another function of forming ears which contact with the surface carrying electrostatic images under the action of a magnet, are performed by the one-component toner in this invention. Accordingly, the composition and particle structure should be arranged to meet the above purpose sufficiently.

The first function of imparting charges to toner particles by friction among them will now be discussed. It is known that if particles of the same substance are frictionally contacted with one another, the attained charges, in general, cannot be large. For example, by simple experiments it was confirmed that the charge quantity obtained by agitating a pulverized resin is smaller than  $10^{-9}$  coulomb/cm<sup>3</sup>, whereas the charge quantity of toner particles forming a developed image by a magnetic brush method, a cascade method or the like is in the order of  $10^{-5}$  coulomb/cm<sup>3</sup>.

The toner per se should have a magnetic property sufficient for the toner particles to perform the other function, namely the function of forming ears having a sliding contact with the surface of an electrostatic latent image under an action of a magnet. For attaining this feature, we incorporate and disperse a fine powder of a magnetic substance into a resin. In this case, since the magnetic substance is used as a toner component, it is preferred that the magnetic substance be black. If its color is not black, it is necessary to incorporate a black pigment such as carbon black into the toner. In view of the foregoing, magnetite (triiron tetroxide) is preferred as the magnetic substance. In preliminary experiments, several kinds of toners were prepared according to the spray drying method by using mixtures of an epoxy resin and magnetite differing in the mixing ratio. As a

result, it was found that when the magnetite content is higher than about 60%, a toner of a such higher magnetite content has generally a better flowability and a better ear-forming property.

Development experiments were carried out by using these toners and a experimental apparatus shown in FIG. 1. In FIG. 1, reference numeral 1 denotes a permanent magnet structure comprising N and S poles arranged alternately and non-magnetic blocks disposed between every two adjacent poles and bonded thereto by an adhesive. A toner 3 is applied on the surface of a plate 2 of a non-magnetic metal such as brass and aluminum. A photosensitive plate 4 is composed of a conductive substrate 6 and a photoconductive layer 5. Electrostatic latent images are formed on the photoconductive layer 5 according to a customary process. A spacer (not shown) is disposed between the metal plate 2 and the photosensitive layer 5 to maintain a clearance of about 1 mm therebetween. During the developing step, the metal plate 2 is slid to the right and left so that ears of the toner have a sliding contact with the surface of a latent image. The photosensitive plate 4 is gradually moved, for example, from the left to the right, so that the entire surface is developed. In this experimental apparatus, several toners were tested by combining them with several photosensitive materials to obtain results shown in Table 1. In this Table, evaluations given on the left column of each photosensitive material are those of the developed images and evaluations given on the right column are those of images transferred on white paper using corona discharge method. In the case of a selenium photosensitive material and an equimolar mixture of polyvinyl carbazole and trinitrofluorenone (PVK/TNF), which provide both positive and negative latent images, the evaluation was conducted with respect to both images. In the Table, evaluation is indicated by symbols , , Δ, and X as implying best quality, satisfactory quality, permissible quality and unsatisfactory quality of the obtained images, respectively.

TABLE 1

| Magnetite Content (%) | Photosensitive Material |        |        |            |             |             |     |
|-----------------------|-------------------------|--------|--------|------------|-------------|-------------|-----|
|                       | ZnO (-)                 | Se (+) | Se (-) | PVK/Se (-) | PVK/TNF (-) | PVK/TNF (+) |     |
| 70 (%)                | ~Δ                      | Δ~X    | Δ~X    | Δ~X        | Δ~X         | Δ~X         | Δ~X |
| 60                    | Δ                       | Δ      | Δ      | Δ          | Δ           | Δ           | Δ   |
| 50                    | Δ                       | X      | X      | X          | X           | X           | X   |
| 40                    | X                       | XX     | XX     | XX         | XX          | XX          | XX  |
| 30                    | XX                      | XXX    | XXX    | XXX        | XXX         | XXX         | XXX |

As is seen from the Table, good results were obtained in the case of a combination of a toner of a magnetite content of 60% and the ZnO photosensitive material, and practically satisfactory results were obtained for a magnetite content ranging from 50% to 65%. In the case of a combination of a toner of a magnetite content of 70% and the ZnO photosensitive material, reduction of the image sharpness by transfer was conspicuous. The reason is considered to be that magnetite particles in the toner particles agglomerate to reduce the specific resistivity of the toner.

Results of an example of measurement of changes in the specific resistivity by the magnetite content are shown in FIG. 2. In general, the specific resistivity of the toner varies depending on the dispersion state, the particle size, the pressure at the time of measurement and the applied voltage, even if the same magnetite and resin are employed and the mixing ratio is kept constant. Accordingly, it must be noted that results shown in FIG. 2 are those under specified conditions. Under

these conditions, the pressure was 1 kg/cm<sup>2</sup>, the applied voltage was 100 V and the thickness of the sample layer was about 4 mm. In this manner, the specific resistivity and the reduction of the image sharpness by transfer were examined. It was found that the specific resistivity should be at least 10<sup>14</sup> Ωcm.

What must be noted among the facts seen from the results shown in Table 1 is that in the case of the Se photosensitive material and the PVK/TNF photosensitive material, the developing effect is substantially the same for both of the cases where latent images are of negative charge and of positive charge. This apparently indicates that positively charged particles and negatively charged particles are present in substantially the same amounts in toner. Images formed on photosensitive materials other than ZnO had a very high edge effect and the image density was not so high in these images. In the case of images formed on the ZnO photosensitive material, black areas could be reproduced in a very good state and no substantial edge effect was observed. However, in the case of a toner of a lower magnetite content, adhesion of the toner was observed around the image, and hair-like protrusion of the toner from contours of the image or roughening of the granularity of the image was conspicuous and the ear-forming ability of the toner was poor. Accordingly, the image was non-uniform and contamination of the image was conspicuous.

When the charge quantity was measured with respect to a toner forming good images on the ZnO photosensitive material, it was found that the charge quantity was about 5 × 10<sup>-6</sup> coulomb/cm<sup>3</sup>. This value is slightly lower than the value obtained in the case of conventional magnetic brush development, but it is much higher than the value obtained in the above-mentioned case where particles of one substance are frictionally contacted with one another. When photos of the toner particles were taken under an electron microscope of about 1000 magnifications, it was found that fine projec-

tions were uniformly distributed on surfaces of the particles and respective projections had a size of about 0.2 to about 0.3 μ.

We drew the following inference from the foregoing observations and the experimental results shown in Table 1.

A vast number of magnetite fine particles are exposed from the surfaces of respective toner particles, and when the magnetite content is about 60%, this exposed state is uniform throughout the entire surfaces. While the prepared toners are stored in a bottle or they are attracted to adhere on the top portion of the magnet at the developing step, they are frictionally in contact with one another and the magnetite present on the particle surfaces are rubbed with the resin, whereby the magnetite will be negatively charged and the resin will be positively charged. The toner as a whole has none of such frictionally developed charges, but respective particles have a vast number of positive and negative

charges on the surfaces thereof and the charges on the entire surfaces of respective particles can be positive or negative. It is believed that particles charged relatively positively are preferably used for developing negatively charged latent images. In general, at the developing step, every time one toner particle is caused to adhere on the latent image, the carrier particles should be deprived of charges of a reverse polarity in correspondence to the charges of said particle. In this invention, however, none of the carrier particles are used, and therefore, when, for example, positively charged particles are caused to adhere to the latent image surface, it is necessary that electrons should be injected into the photosensitive layer from the magnetite faces of the negatively charged particles (since the toner has insulating properties, charges are not allowed to move along ears of the toner). In case positively charged images are developed, every time one negatively charged particle is caused to adhere to the latent image surface, it is necessary that an electron is injected into the magnetite of the corresponding adjacent positive particle from the photosensitive layer to thereby deprive the positive particle of the charge. In a zinc oxide photosensitive material, the above mechanism is allowed to proceed very smoothly, and the charge distribution on the surface of the photosensitive layer is microscopically non-uniform. Accordingly, the intensity of the surface electric field is enhanced. For these reasons, it is construed that especially good results are obtained when a zinc oxide photosensitive material is used.

The foregoing can be summarized as follows:

1. Respective toner particles comprises fine particles of a magnetic substance dispersed in a resin, and faces of the magnetic substance particles are exposed.
2. The magnetic substance is negatively charged by frictional contact with the resin (the resin is positively charged).
3. A ZnO-resin dispersion layer is used as a photosensitive layer.
4. N and S poles arranged alternately, a non-magnetic plate, a toner adhering theron and a photosensitive plate having contact with tips of ears of the toner are disposed in this order, and a relative movement is conducted between the magnetic poles and the metal plate.

These matters will now be expatiated.

The magnetic substance to be used in this invention should satisfy the foregoing requirements 1 and 2, and it is also required that it should be deprived of negative charges by injection of electrons into the ZnO photosensitive layer. Therefore, the magnetic substance should be a conductor or semiconductor of the electronic conduction type. Since it is required that the toner should be black, if the magnetic substance is not black, carbon black or other black dye or pigment should be added, resulting frequently in bad influences on the electric resistance and the triboelectric chargeability. Accordingly, it is considered preferable for the magnetic substance to be black, have a good dispersibility in the resin, be chemically stable and be easily formed in fine particles having a size not exceeding  $1\mu$ . Magnetite satisfies substantially all of these conditions, and it is used most preferably as the magnetic substance in this invention. Of course, fine particles of various ferrites, iron, cobalt and nickel can be used when combined with appropriate resins.

The resin to be used in this invention is chosen with regard to the chargeability on friction with the mag-

netic substance used, the manufacturing process and conditions, the covering property to the magnetic substance, the adaptability to thermal fixation and other factors. Styrene resins, acrylic resins, vinyl resins, epoxy resins, cellulose resins, polyurethane resins and copolymers thereof are appropriately chosen and used. They are used singly or in the form of a mixture of two or more of them.

The toner of this invention is prepared from an appropriate combination of the magnetic substance and resin as mentioned above according to a known toner-preparing process. A most popular process for preparing toners comprises heating and kneading a resin and a pigment by two rollers and pulverizing the resulting mixture. There is also known a spray-drying process such as disclosed in the specification of U.S. Pat. No. 3,338,991.

As pointed out repeatedly hereinbefore, it is an indispensable requirement that fine particles of the magnetic substance are exposed on the surfaces of the toner particles, and it is important that the toner is prepared so that this requirement is satisfied in the resulting toner. This condition is greatly influenced by the kinds of the magnetic substance and resin to be used and the content of the magnetic substance. In the spray-drying process, as the dispersion state is better, the particles of the magnetic substance are better covered with the resin, and as the amount of the solvent is smaller, the disc rotation number is larger and feeding air temperature is lower, a better coating is obtained. If the degree of exposure of the particles of the magnetic substance is too high, the specific resistivity of the toner is lowered and the triboelectric charge quantity of each particle cannot become large. Accordingly, it is necessary to take care so that the degree of exposure is not too high.

All of commercially available zinc oxide photosensitive materials used for copying machines of the electrofax type can be used as the zinc oxide photosensitive material in this invention. Since this invention is directed to the transfer of developed images on ordinary papers, use of zinc oxide photosensitive materials to be used for PPC (plane paper copiers) is preferred, and a commercially available master paper for a U-bix copying machine (manufactured by Konishiroku Photo Industry Co., Ltd.) is a most preferred example of such photosensitive material.

FIG. 1 is a view illustrating the principle of the apparatus to be used for carrying out the developing method of this invention.

FIG. 2 is a diagram showing the relation between the electric resistivity of the toner and the content of a magnetic substance in the toner. FIG. 3 shows one embodiment of the development apparatus to be used for working the developing method of this invention. FIGS. 4 and 5 show another embodiments of the developing apparatus to be used for working the developing method of this invention.

A developing device having a principle as shown in FIG. 1 is preferably employed in this invention. The intended object of this invention can be attained even if magnetic poles are not strictly disposed in N-S alternating arrangement. Further, the development can be performed even if magnetic poles 1 and metal plate 2 are fixed to each other and they are integrally moved, though the image quality is reduced to some extent. Since the apparatus shown in FIG. 1 is an experimental apparatus, in an actual operation a modification should be made so that feeding of the toner onto the metal plate and movement of the metal plate can be performed

continuously. An example of such modification is illustrated in FIG. 3.

In FIG. 3, reference numerals 7 and 3 denote a toner vessel and a toner, respectively, and the toner 3 is fed onto a surface carrying electrostatic images from the toner vessel 7 by a toner feeder 9 and is subjected to the development treatment. The feeder 9 comprises a non-magnetic cylinder 10 and a permanent magnet 11 disposed in the interior of the cylinder and including N and S poles arranged alternately. A zinc oxide photosensitive layer 13 is coated on a drum type substrate 14. 1 indicates a toner layer, and when the metal cylinder 10 is rotated in a direction indicated by an arrow, the toner 3 is attracted from the toner vessel 7 through a clearance formed between a regulating plate 12 and the peripheral face of the cylinder 10 by the attracting force of the magnetic poles 11. In FIG. 3, the toner layer 1 is drawn as though it has a uniform thickness, but actually, ears rise at parts confronting the centers of the respective poles while other portions of the toner layer 1 remain flat. Even if positions of the magnetic poles are slightly deviated in the vertical direction by rotating and moving them entirely, development can be performed.

FIG. 4 illustrates another preferred embodiment of 25 the apparatus used in this invention. A developing roller 15 comprises a core 16 composed of a non-magnetic material such as aluminum or brass and a number of magnets 17 disposed on its outer peripheral face. A toner 3 is charged in a toner vessel 18, and when the 30 developing roller 15 is rotated in a direction indicated by an arrow A, the toner is held on the magnets 17 by the attractive force thereof and is withdrawn from the toner vessel 18 as the developing roller 15 is rotated. When N and S poles are arranged alternately as is 35 shown in FIG. 4, the toner is held between every two adjacent poles by the action of the lines of magnetic force, and the toner ears in a brush-like form appear on the magnet 17 where the lines of magnetic force are vertically upwardly directed. If a mutual relation between the developing roller 15 and the photosensitive material 20 is established so that the eared toner is allowed to have a sufficient contact with the photosensitive material 20, an electrostatic latent image 21 on the photosensitive material 20 advancing in a direction 40 indicated by an arrow B is developed to form a toner image 22. Development on portions other than ears causes fogs, and accordingly it is preferred that the development be performed only on earing portions. Uneven development caused by the presence of clearances between two adjacent ears can be prevented sufficiently if the developing roller 15 is rotated at a peripheral speed several times the peripheral speed of the photosensitive material 20. The advantage attained in this embodiment is that since the toner is held directly 45 by the magnet 17, a high magnetic force can be utilized and development can be performed stably, and that the structure is simpler than that of an apparatus of the sleeve type.

In FIG. 4, magnets of N and S polarities are arranged 50 alternately, but in this embodiment, since development is performed by eared portions alone and these eared portions are held directly on the magnets, they need not be arranged in such N-S alternating relationship.

Still another embodiment of the apparatus used in this 55 invention is illustrated in FIG. 5.

A photosensitive plate 24 is disposed at a central flat portion of a supporting basin 23 composed of a non-

magnetic substance, and left and right side portions of the supporting basin 23 form toner vessels 26 in which a toner 3 is filled. A charger 28 and an exposure slit 29 are moved over the photosensitive material 24 in a direction indicated by an arrow C to form an electrostatic latent image, and then a magnet 30 is moved under the back surface of the photosensitive material 24 in a direction indicated by an arrow D and development takes place with the toner 3 held by the magnet 30 through the photosensitive material 24 and the supporting basin 23.

According to the method of this invention using a toner 3 and a photosensitive material 24 in combination, even if electrodes confronting to the zinc oxide photosensitive material 24 are not disposed, solid and clear images free of an edge effect can be obtained by the above development procedures.

The magnet 30 is so arranged that it is moved while facing the supporting basin 23. Accordingly, the toner 3 withdrawn from the left vessel 26 is charged in the right vessel 26' and it is then returned to the left vessel 26. The top ends 31 and 31' of the vessels 26 and 26' form ear height-regulating plates for controlling the height of ears attracted to the magnet 30.

Apparatuses shown in FIGS. 3, 4 and 5 are embodiments of the apparatus to be used for practising the method of this invention, and as is apparent to those skilled in the art, various modifications may be made based on the principle illustrated in FIG. 1.

The invention will now be illustrated in detail by reference to the following Examples.

#### EXAMPLE 1

|                                                                 |        |
|-----------------------------------------------------------------|--------|
| Epon 1004 (epoxy resin manufactured by Shell Chemical)          | 240 g  |
| Mapico Black (triron tetroxide manufactured by Columbia Carbon) | 360 g  |
| Toluene                                                         | 280 g  |
| Acetone                                                         | 120 g  |
| Total                                                           | 1000 g |

The above composition was dispersed for 32 hours in a porcelain ball mill and then granulated according to the spray drying method using a rotary disc. The spray drying conditions were as follows:

|                                 |        |
|---------------------------------|--------|
| Solvent:                        |        |
| toluene                         | 1680 g |
| acetone                         | 720 g  |
| Non-volatile solids:            |        |
| 600 g                           |        |
| Rotation number of rotary disc: |        |
| 44,000 r.p.m.                   |        |
| Drying air temperature:         |        |
| 170° C.                         |        |

Thus, there were obtained black spherical toner particles having an average particle size of about 10 $\mu$ .

A copying machine U-bix 800 (manufactured by Konishiroku Photo Industry Co., Ltd.) of which a developing device was taken out, was used. First, a copy button was depressed and when formation of an electrostatic image on a master paper was completed, a power switch was put off to stop the machine. A master paper was taken out under safety light, and development was carried out with the above toner by using an apparatus based on the principle shown in FIG. 1. Then, the mas-

ter paper was set in the machine again, and after charging and exposure devices had been inactivated, the copy button was depressed and the developed image was transferred to an ordinary paper. A good image was obtained.

## EXAMPLE 2

|                                                                                 |        |    |
|---------------------------------------------------------------------------------|--------|----|
| Pliolite ACL (styrene-acrylic acid copolymer manufactured by Goodyear Chemical) | 240 g  | 5  |
| Mapico Black (triiiron tetroxide manufactured by Columbia Carbon)               | 360 g  | 10 |
| Toluene                                                                         | 280 g  | 15 |
| Acetone                                                                         | 120 g  |    |
| Total                                                                           | 1000 g |    |

The above composition was dispersed in a porcelain ball mill for 16 hours and granulated according to the spray drying method using a rotary disc. The spray 20 drying conditions were as follows:

|                                 |        |    |
|---------------------------------|--------|----|
| Solvent:                        |        | 25 |
| toluene                         | 1260 g |    |
| acetone                         | 540 g  |    |
| Non-volatile solids:            |        |    |
| 600 g                           |        |    |
| Rotation number of rotary disc: |        |    |
| 49,000 r.p.m.                   |        |    |
| Drying air temperature:         |        |    |
| 190° C.                         |        |    |

Thus, there were obtained black spherical toner particles having an average particle size of about 10 $\mu$ , and when an image was formed by using the so prepared 35 toner in the same manner as described in Example 1, good results were obtained.

## EXAMPLE 3

|                                                                         |        |    |
|-------------------------------------------------------------------------|--------|----|
| Pentaly A (rosin ester of pentaerythritol manufactured by Hercules Co.) | 240 g  | 40 |
| Mapico Black                                                            | 360 g  |    |
| Toluene                                                                 | 280 g  |    |
| Acetone                                                                 | 120 g  |    |
| Total                                                                   | 1000 g |    |

The above composition was dispersed for 4 hours in a porcelain ball mill and granulated according to the spray drying method using a rotary disc. The spray 50 drying conditions were as follows:

|                                 |        |    |
|---------------------------------|--------|----|
| Solvent:                        |        | 45 |
| toluene                         | 1680 g |    |
| acetone                         | 720 g  |    |
| Non-volatile solids:            |        |    |
| 600 g                           |        |    |
| Rotation number of rotary disc: |        |    |
| 44,000 ppm                      |        |    |
| Drying air temperature:         |        |    |
| 170° C.                         |        |    |

Thus, there were obtained black spherical toner particles having an average particle size of about 10 $\mu$ , and in the same manner as described in Example 1, development was conducted by using the so prepared toner and the developed image was transferred. An image of good quality was obtained.

## EXAMPLE 4

|                                                                                   |        |
|-----------------------------------------------------------------------------------|--------|
| Piccolastic C125 (styrene resin manufactured by Pennsylvania Industrial Chemical) | 168 g  |
| Piccovar 450H (polyindene resin manufactured by Pennsylvania Industrial Chemical) | 72 g   |
| Mapico Black                                                                      | 360 g  |
| Toluene                                                                           | 280 g  |
| Acetone                                                                           | 120 g  |
| Total                                                                             | 1000 g |

The above composition was dispersed for 17.5 hours in a porcelain ball mill, and then granulated according to the spray drying method using a rotary disc. The spray drying conditions were as follows:

|                                 |        |    |
|---------------------------------|--------|----|
| Solvent:                        |        | 25 |
| toluene                         | 1260 g |    |
| acetone                         | 540 g  |    |
| Non-volatile solids:            |        |    |
| 600 g                           |        |    |
| Rotation number of rotary disc: |        |    |
| 49,000 r.p.m.                   |        |    |
| Drying air temperature:         |        |    |
| 190° C.                         |        |    |

Thus, there were obtained black spherical toner particles having an average particle size of about 10 $\mu$ . In the same manner as described in Example 1, development was carried out by using the so prepared toner and the developed image was transferred. An image of good quality was obtained.

As a result of experiments made separately, it was confirmed that each of the resins used in the foregoing Examples was positively charged by frictional contact with magnetite (Mapico Black). Further, from electron microscope photographs of toners obtained in the foregoing Examples it was confirmed that fine convexities having a size corresponding to the size of magnetite particles were uniformly distributed on the surfaces of the toner particles.

## EXAMPLE 5

|              |        |
|--------------|--------|
| Pliolite ACL | 400 g  |
| Mapico Black | 600 g  |
| Total        | 1000 g |

The above composition was kneaded at 65° C. for 10 minutes by means of a two-roll mill and ground by a jet grinder. Then, the ground product was granulated for 16 hours together with 500 g in a porcelain ball mill and dried for 1 week in an air current maintained at 40° C.

55 Then, the resulting powder was sprayed and injected in a drier by a bi-fluid type nozzle and made spherical by feeding hot air (190° C.) in the drier. Thus, there were obtained black spherical toner particles having an average particle size of about 10 $\mu$ . In the same manner as described in Example 1, development was carried out by using the so prepared toner and the developed image was transferred. An image of good quality was obtained.

Each of the toners used in the foregoing five Examples was composed of spherical particles. However, in this invention it is not a critical requirement that toner particles should have a spherical form. As a result of our experiments, it was confirmed that spherical toners

have generally better flowability than pulverized non-spherical toners. Of course, some of pulverized non-spherical toners were found to have a sufficient flowability and they could be effectively used in this invention directly in the pulverized state. No definite critical value is found as regards the flowability, but particles having a Carr flowability index lower than 30 are not suitable and use of particles having a Carr flowability index higher than 50 is preferred.

In the foregoing illustration, the triboelectric chargeability of the resin used in the toner of this invention have been discussed with respect to the magnetic substance alone. Through our experiments, we empirically found the following facts as regards the triboelectric chargeability of the toner of this invention with respect to the photosensitive layer.

As shown in Table 2 given hereinafter, when 8 toners A to H were tested on the triboelectric chargeability to the photosensitive layers, it was found that 4 toners A to D were positively charged and another 4 toners E to H were negatively charged. When images were formed by using these toners in the same manner as in the preceding Examples, it was found that transferred images formed by using toners A to D were a little superior to transferred images formed by using toners E to H in the image quality, namely the image density and sharpness.

Most of resins have a negative triboelectric chargeability to ZnO photosensitive layers, and magnetite has also a negative triboelectric chargeability to ZnO photosensitive layers. However, when magnetite alone is compression-molded and the resulting mass is rubbed with a ZnO photosensitive material, it is seen that the magnetite is negatively charged but the charge quantity is very small and is substantially zero. Accordingly, it is believed that the triboelectric chargeability of the toner of this invention to the photosensitive layer depends mainly on properties of the resin. Toners A to D are those prepared by incorporating in a resin a charge controlling agent such as Nigrosine or a polymer or oligomer having a highly electron-donative functional group such as an amino group. Details of preparation of toners of this type will be apparent from Example 6 given hereinafter.

TABLE 2

| Kind of Toner | Triboelectric Chargeability to Photosensitive Layer | Image Quality |
|---------------|-----------------------------------------------------|---------------|
| A             | +                                                   |               |
| B             | +                                                   |               |
| C             | +                                                   |               |
| D             | +                                                   |               |
| E             | -                                                   |               |
| F             | -                                                   |               |
| G             | -                                                   |               |
| H             | -                                                   |               |

## EXAMPLE 6

|               |        |
|---------------|--------|
| Epon 1004     | 222 g  |
| Mapico Black  | 360 g  |
| Nigrosine SSB | 18 g   |
| Toluene       | 280 g  |
| Acetone       | 120 g  |
| Total         | 1000 g |

The above composition was dispersed for 16 hours in a porcelain ball mill and granulated by the spray drying

method using a rotary disc. The spray drying conditions were as follows;

|    |                                 |        |
|----|---------------------------------|--------|
| 5  | Solvent:                        |        |
|    | toluene:                        | 1680 g |
|    | acetone:                        | 720 g  |
|    | Non-volatile solids:            |        |
|    | 600 g                           |        |
| 10 | Rotation number of rotary disc: |        |
|    | 44,000 r.p.m.                   |        |
|    | Drying air temperature:         |        |
|    | 170° C.                         |        |

Thus, there were obtained black spherical toner particles having an average particle size of  $10\mu$ . In the same manner as described in Example 1, development was carried out by using the so prepared toner and the developed image was transferred. The quality of the resulting image was slightly improved over the quality of the image obtained in Example 1.

From the foregoing illustration, those skilled in the art will readily understand the concept, structural requirements and working of this invention and from the foregoing Examples they will readily anticipate other similar embodiments of the method of this invention.

What we claim is:

1. A method for forming a toner image on a photosensitive material bearing an electrostatic latent image comprising
  - (a) introducing a one component developer consisting of fine toner particles, said particles containing a resin and ferromagnetic powder dispersed in said resin in such a fashion that a portion of said ferromagnetic powder is exposed on the surface of said toner particles, said toner particles having a specific resistivity of at least  $10^{14}$  ohm cm and being capable of accepting a triboelectric charge, into a toner vessel which includes a regulating plate for controlling the amount of toner to be fed,
  - (b) feeding said toner onto a toner feeder comprising a non-magnetic cylinder drum and a plurality of magnets disposed therein so that south and north poles are directed to the inner surface of non-magnetic cylinder,
  - (c) carrying said toner, by rotary movement of either said non-magnetic cylinder or said plurality of magnets, along the surface of said non-magnetic cylinder into close proximity to said electrostatic latent image,
- 50 5. said toner particles developing a triboelectric charge of a polarity opposite to that of said electrostatic latent image during steps (a) through (c) in the absence of a corona discharging device, and
  - (d) bringing said toner particles into contact with said electrostatic latent image.
2. The method of claim 1 wherein said toner particles have been produced by a spray-drying process.
3. The method of claim 1 wherein said triboelectric charge is developed by virtue of mutual friction between toner particles.
4. The method of claim 1 wherein said ferromagnetic material is comprised of fine particles of ferrite.
5. The method of claim 4 wherein said ferromagnetic material is magnetite.
6. The method of claim 5 wherein said magnetite content is greater than 50%.
7. The method of claim 1 wherein said resin is selected from the group consisting of styrene resins,

acrylic resins, vinyl resins, epoxy resins, cellulose resins, polyurethane resins, copolymers thereof, and mixtures thereof.

8. The method of claim 1 wherein said ferromagnetic

material comprises particles of a size not exceeding one micron.

9. The method according to claim 1 wherein said toner particles are formed with fine projections having a size of 0.2 to 0.3 microns.

\* \* \* \* \*

10

15

20

25

30

35

40

45

50

55

60

65